



US006599390B2

(12) **United States Patent**  
Rheims et al.

(10) Patent No.: US 6,599,390 B2  
(45) Date of Patent: Jul. 29, 2003

- (54) **PROCESS FOR LOADING FIBERS WITH CALCIUM CARBONATE IN A PLURALITY OF REACTORS**

(75) Inventors: **Jörg Rheims**, Heidenheim (DE); **Klaus Doelle**, Menasha, WI (US); **Oliver Heise**, Menasha, WI (US); **Werner Witek**, Appleton, WI (US)

(73) Assignee: **Voith Paper Patent GmbH**, Heidenheim (DE)

(\*) Notice: Subject to any disclaimer, the term of this patent is extended or adjusted under 35 U.S.C. 154(b) by 0 days.

(21) Appl. No.: 09/903,975

(22) Filed: Jul. 12, 2001

(65) **Prior Publication Data**

US 2002/0007925 A1 Jan. 24, 2002

(30) Foreign Application Priority Data

Jul. 13, 2000 (DE) ..... 100 33 978

(51) Int. Cl.<sup>7</sup> ..... D21H 11/16; I

(52) U.S. Cl. .... 162/9; 162/181.2; 162/182;  
162/183; 162/241

(56) **References Cited**

## U.S. PATENT DOCUMENTS

3,849,247 A \* 11/1974 Richter ..... 162/237

- |      |                                                                                                                                                                           |              |   |         |                       |           |
|------|---------------------------------------------------------------------------------------------------------------------------------------------------------------------------|--------------|---|---------|-----------------------|-----------|
| (54) | <b>PROCESS FOR LOADING FIBERS WITH CALCIUM CARBONATE IN A PLURALITY OF REACTORS</b>                                                                                       | 4,431,480 A  | * | 2/1984  | Markham et al. ....   | 162/19    |
|      |                                                                                                                                                                           | 4,842,690 A  | * | 6/1989  | Gazdik et al. ....    | 162/57    |
|      |                                                                                                                                                                           | 5,096,539 A  |   | 3/1992  | Allan .....           | 162/9     |
|      |                                                                                                                                                                           | 5,223,090 A  | * | 6/1993  | Klungness et al. .... | 162/9     |
| (75) | Inventors: <b>Jörg Rheims</b> , Heidenheim (DE); <b>Klaus Doelle</b> , Menasha, WI (US); <b>Oliver Heise</b> , Menasha, WI (US); <b>Werner Wittek</b> , Appleton, WI (US) | 5,665,205 A  |   | 9/1997  | Srivatsa et al. ....  | 162/181.4 |
|      |                                                                                                                                                                           | 5,679,220 A  |   | 10/1997 | Matthew et al. ....   | 162/181.4 |
|      |                                                                                                                                                                           | 6,264,794 B1 |   | 7/2001  | Neumann et al. ....   | 162/205   |

## FOREIGN PATENT DOCUMENTS

EP 0 457 235 A1 5/1991 ..... D21H/17/70  
 EP 0 791 685 A2 8/1997 ..... D21H/17/70  
 WO WO 97/01670 1/1997 ..... D21H/17/67

#### OTHER PUBLICATIONS

Fogler, "Chemical rxn Engineering", FAQ, Chapter 4, University Michigan.\*

\* cited by examiner

*Primary Examiner*—Steve Alvo

(74) *Attorney, Agent, or Firm*—Taylor & Aust, P.C.

(57) **ABSTRACT**

For a process and an apparatus for loading fibers contained in a pulp suspension with calcium carbonate, a calcium oxide and/or a medium containing calcium hydroxide is fed to the pulp suspension, and the so treated pulp suspension is further charged in several reactors with pure carbon dioxide or a medium containing carbon dioxide. The reactors can be connected in series and/or in parallel. The reactor can produce different forms of calcium carbonate.

## 2 Claims, 1 Drawing Sheet





**PROCESS FOR LOADING FIBERS WITH  
CALCIUM CARBONATE IN A PLURALITY  
OF REACTORS**

**BACKGROUND OF THE INVENTION**

1. Field of the Invention

The invention concerns a process for loading fibers contained in a pulp suspension with calcium carbonate.

2. Description of the Related Art

Pulp suspensions of the above-mentioned type are used especially in paper and cardboard manufacture. The sparing use of raw material resources, due especially to economical and ecological concerns, is reflected in the paper production industry by the use of paper web with lower basis weights, as well as by the partial replacement of pulp with filling materials. If lower cost raw materials are used, the paper quality should at least be maintained. Among other things, the end product's strength, visual characteristics, and processability play key roles in this challenge.

**SUMMARY OF THE INVENTION**

The present invention relates to a process and apparatus for loading fibers with calcium carbonate, especially in terms of optimum reaction balance, optimum reaction speed and optimum flexibility of production output.

The invention comprises, in one form thereof, a process of fiber loading that includes adding calcium oxide and/or a medium containing calcium hydroxide to a pulp suspension, and then charging the pulp suspension in several reactors with pure carbon dioxide or a medium containing carbon dioxide. Upon the addition of calcium oxide and/or a medium containing calcium hydroxide to the pulp, an exothermic chemical reaction takes place, the calcium hydroxide being added in liquid form (lime milk). By using lime milk, the water settled in or on the pulp suspension's fibrous material is not necessarily required to start and continue the chemical reaction.

Because of this development, the chemical process, which is the basis of the loading, is split into several small processes, thereby permitting an optimum reaction balance, an optimum reaction speed, and an optimum flexibility of production output to be achieved. This use of several small processes enables a targeted and optimal testing of partial reactions, switching on and off of partial reactors and a variation of the operating parameters in the partial reactors.

On loading the fibers, calcium carbonate is imbedded into the wetted fiber surfaces by adding calcium oxide and/or calcium hydroxide to the wet fibrous material. Thereby, at least part of this calcium compound can associate with the water of the pulp mass. The so treated fibrous material is then charged with the pure carbon dioxide or the medium containing carbon dioxide.

As a result, the term "wetted fiber surface" can include all wetted surfaces of the individual fibers. Consequently, the fibers become loaded with calcium carbonate both on their outer surfaces and on their insides (lumen).

Accordingly, the fibers are loaded with the filler material calcium carbonate, whereby the accumulation on the wetted surfaces takes place by a so-called "Fiber Loading™" process, as described in U.S. Pat. No. 5,223,090. In this "Fiber Loading™" process, the carbon dioxide reacts with the calcium hydroxide to form water and calcium carbonate.

For one suitable arrangement of the process in conformity with the invention, at least one section of the reactor is

connected in series. Several smaller reaction volumes are created from one large reaction volume, so that the reaction speed is increased and, correspondingly, the contact surfaces of the reactants are enlarged. Furthermore, in an advantageous manner, (crystallization-) processes can be achieved in a targeted fashion and the parameters for an optimal reaction can be matched.

With a further advantageous arrangement, at least one section of the reactors is connected in parallel. In addition to the above-mentioned advantages, this arrangement also allows for optimum adaptability of the production output. It is also of advantage, in parallel-connected reactors, to produce calcium carbonate with different crystal types and, preferably, to mix these on termination of the production process. This mixing allows an optimal composition of the product.

In certain cases, a combination of series- and parallel-connection of the reactors are of benefit. In this way, the parallel section can be matched to the required production range.

In other respects, the loading of fibers with calcium carbonate is as described in U.S. Pat. No. 5,223,090. The content of that patent is hereby incorporated by reference herein.

The apparatus embodying the invention essentially includes several reactors, in which the pulp suspension, mixed with calcium oxide and/or calcium hydroxide, can be charged with pure carbon dioxide or a medium containing carbon dioxide.

**BRIEF DESCRIPTION OF THE DRAWINGS**

The above-mentioned and other features and advantages of this invention, and the manner of attaining them, will become more apparent and the invention will be better understood by reference to the following description of an embodiment of the invention taken in conjunction with the accompanying drawing, wherein:

FIG. 1 is a schematic illustration of an embodiment of the fiber loading apparatus of the present invention.

The exemplification set out herein illustrates one preferred embodiment of the invention, in one form, and such exemplification is not to be construed as limiting the scope of the invention in any manner.

**DETAILED DESCRIPTION OF THE  
INVENTION**

FIG. 1 shows in schematic an apparatus 10 for loading fibers, contained in a pulp suspension, with calcium carbonate ( $CaCO_3$ ). Correspondingly, apparatus 10 serves to add the calcium carbonate to the wetted fiber surfaces of the fibrous material. In this way, this loading of the fibers, especially in accordance with the aforementioned "Fiber Loading™" process, takes place.

Apparatus 10 includes several reactors 12, in which the pulp suspension, mixed with calcium oxide ( $CaO$ ) and/or calcium hydroxide ( $Ca(OH)_2$ ) can be charged by pure carbon dioxide ( $CO_2$ ) or by a medium containing carbon dioxide ( $CO_2$ ). Moreover, reactors 12, can be connected in series or parallel. It is possible to have a series arrangement, a parallel arrangement, or a combination arrangement of series and parallel for reactors 12. Also, with parallel-connected reactors 12, it is possible to produce calcium carbonate with different types of crystal and to mix these, preferably on termination of the respective production process.



What is claimed is:

1. A process for loading calcium carbonate into fibers contained in a pulp suspension, the process comprising the steps of:
  - providing a pulp suspension comprised of fibers;
  - providing a calcium-rich medium, said calcium-rich medium being comprised of at least one of calcium oxide and calcium hydroxide;
  - adding said calcium-rich medium to said pulp suspension to form a calcium-treated pulp suspension;
  - providing a plurality of reactors, wherein said plurality of reactors includes at least one section of reactors, said at least one section of reactors being connected in parallel, each reactor being fluidly coupled to a source of a carbon-dioxide medium, said carbon-dioxide medium

being one of pure carbon dioxide and a medium containing carbon dioxide;  
charging said calcium-treated pulp suspension and said carbon-dioxide medium into at least one reactor to promote a chemical reaction to form calcium carbonate and thereby load said fibers with said calcium carbonate; and  
producing a different crystalline form of calcium carbonate in each of said parallel-connected reactors; and  
mixing together said different crystalline forms of calcium carbonate.

2. The processes of claim 1, wherein said mixing step occurs after the production of all of said different crystalline form of calcium carbonate being formed is complete.

\* \* \* \* \*

UNITED STATES PATENT AND TRADEMARK OFFICE  
**CERTIFICATE OF CORRECTION**

PATENT NO. : 6,599,390 B2  
DATED : July 29, 2003  
INVENTOR(S) : Rheims et al.

Page 1 of 1

It is certified that error appears in the above-identified patent and that said Letters Patent is hereby corrected as shown below:

Title page.

Item [56], **References Cited**, FOREIGN PATENT DOCUMENTS, please add the following -- GB 2 265 916 A 10/1993 ....D21H/15/02 --;  
OTHER PUBLICATIONS, please add the following -- Klungness, J.H., et al.: Fiber Loading: Progress Report. In: Recycling Symposium Proceedings (TAPPI), May 15-18, 1994, S 283-290, AN 94:3519 PAPERCHEM2. --; and  
Item [57], **ABSTRACT**,  
Line 7, please delete "reactor", and substitute therefore -- reactors --.

Signed and Sealed this

Thirteenth Day of July, 2004



JON W. DUDAS  
*Acting Director of the United States Patent and Trademark Office*